

Oct. 6, 1959

S. TOUR

2,907,637

## PROCESS OF WINNING ELEMENTAL PHOSPHORUS

Filed Oct. 5, 1955

2 Sheets-Sheet 1



INVENTOR

BY Arnold Sprung

ATTORNEY

Oct. 6, 1959

S. TOUR

2,907,637

PROCESS OF WINNING ELEMENTAL PHOSPHORUS

Filed Oct. 5, 1955

2 Sheets-Sheet 2



INVENTOR  
SAM TOUR

BY

*Arnold Sprung*

ATTORNEY

1

2,907,637

## PROCESS OF WINNING ELEMENTAL PHOSPHORUS

Sam Tour, New York, N.Y., assignor to Louis Burgess and himself; Murray Burgess and Eddie Burgess Beiter, executors of the estate of said Louis Burgess, deceased

Application October 5, 1955, Serial No. 538,597

12 Claims. (Cl. 23—223)

This invention is a new and useful process of winning elemental phosphorous from oxygenated ores containing the same, such as the so-called phosphate rock. The invention is an improvement on the method described and claimed in application of Louis Burgess, Serial No. 530,507, filed August 25, 1955, the said application and the instant application being assigned to the identical assignee. This invention will be fully understood from the following description read in conjunction with the drawings in which:

Fig. 1 is a diagrammatic vertical section thru apparatus in which the invention may be practiced;

Fig. 2 is a detailed vertical section through one element of the apparatus shown in Fig. 1;

Fig. 3 is a horizontal section through the plane indicated by 3—3 in Fig. 2; and

Fig. 4 is a horizontal section through the plane indicated by 4—4 in Fig. 2.

The elements of the process for the recovery of elemental phosphorus described in said application, Serial No. 530,507, are as follows:

(a) The formation of a coke throughout which the particles of the ore are disseminated in a supporting structure of carbon and in which the carbon is in excess of that consumable by reduction of the ore and other reducible substances present;

(b) Heating the coke so formed out of direct contact with combustion gases to a temperature at which the ore is reduced by carbon thereby producing elemental phosphorus and carbon monoxide in vapor phase, conducting away the vapor phase and condensing the phosphorus;

(c) Removing the residue of excess carbon and inorganic oxides from the heating zone in solid form.

The substantially complete liberation of the elemental phosphorus in step (b) and the removal of the residue in solid form, step (c), are made possible by the preliminary step (a), i.e., the formation of a coke in which the particles are disseminated and in which the carbon is in excess. The combined effect of the coke structure and the excess carbon in this coke structure is to hold the oxide particles apart up to the point of complete reduction and at this point, to provide sufficient residual carbon to hold the residual oxide particles apart and thereby prevent sintering. In the preferred embodiment, sufficient excess carbon is incorporated to maintain the physical form of the individual masses of which the charge is composed.

In one method of generating the desired coke structure, the oxide is mixed with sufficient of a substance selected from the tars, pitches, and asphalts (including the oxidized asphalts), to occupy the spaces between the oxide particles. Sufficient coke breeze, anthracite

2

or bituminous coal of about the same particle size as the oxide particles, is also incorporated in amount sufficient to provide the requisite carbon:oxide ratio. In another method, the oxide and bituminous coal, are ground together in a state of extreme fineness for a period of several hours. The grinding is continued until the individual particles of oxide and coal are no longer separately distinguishable and the coal has acquired the property of flowing under extreme pressure. At this stage, the entire mix is briquetted by the application of pressures of the order of at least ten tons per square inch.

In either method, the coke-forming substance is converted into coke by raising the temperature progressively through the range of pyrolysis, i.e., about 350—1000° C., until pyrolysis is substantially complete. With coke-forming substances that become fluid below the temperature of pyrolysis, this heating is carried out in apparatus in which the mix is supported in a quiescent state, such as a coke oven or broad oven. With those coke-forming substances which become only plastic and not freely fluid up to the temperature of pyrolysis, the carbonization may be carried out in a vertical retort with top feed and bottom discharge.

Any of the coke-forming substances mentioned may, with sufficiently rigorous preliminary treatment, be converted into forms that become only plastic and not freely fluid up to the temperature of pyrolysis. Those predominantly suited for this purpose are, however, the coal tar pitches of about 100° C. or higher melting point, as determined by the cube in air method and the bituminous coals processed in the manner hereinabove described. It is to this embodiment of the invention described in said application, Serial No. 530,507, that my improvement is directed.

Referring to the drawings, 1 designates a retort of the vertical type, with provision for top feed and bottom discharge. By reference to Fig. 2 which shows details of construction, heating zone 2 is bounded by transverse walls 3 and 4 and end walls 5 and 6 (Figs. 3 and 4). These are of refractory heat-conducting material, such as fused alumina or bonded silicon carbide.

Wall 4 is heated by the application of combustion gases to surface 7 thereof. For this purpose, burner 8 is provided which may be supplied with air and gas through the valved pipes 9 and 10 respectively. Burner 8 discharges into combustion space 11 defined by the refractory panels 12, 13 and 14. From the combustion space, the products of combustion move upwardly through duct 15 defined by the refractory walls 4, 5, 6 and 16. They follow a sinuous path over the staggered horizontal baffles 17 as indicated by arrows 18, eventually passing out through the stack 19, by which they are discharged.

Transverse wall 3 is heated by the application of combustion gases to surface 20 thereof. For this purpose, burner 21 is provided which may be supplied with air and gas through valved pipes 22 and 23. The burner discharges into combustion space 24 defined by the refractory panels 25, 26 and 27. From the combustion space 24, the products of combustion move upwardly through duct 28 defined by the refractory walls 3, 5, 6 and 29. They follow a sinuous path over staggered baffles 30 as indicated by arrows 31 passing off through the stack 32 by which they are discharged.

Material to be supplied to heating zone 2 is dumped

into hopper 33 from which by operation of bell valve 34 it may be discharged into hopper 35, from which by operation of bell valve 36, it may be discharged into heating zone 2.

This makes it possible to introduce charge into heating zone 2 without releasing the pressure which obtains therein. In practice, the heating zone 2 is operated with charge up to about the level indicated by the line 37.

Charge may be continuously withdrawn from the lower end 38 of heating zone 2 by means of turnable grate bars 39. The grate bars are rotated preferably continuously, by any suitable means, not shown. Material discharged by grate bars 39 drops into space 41 from which it may be continuously or intermittently removed by the operation of worm conveyor 42. A carrier gas may be introduced into space 41 through valved pipe 43.

Provision is made for the take-off of gases from adjacent the upper part of heating zone 2 through the horizontal ducts 44 and 45 (Figs. 2 and 3) discharging into the main 46 controlled by valve 47. Provision is also made for the take-off of gases from a mid-point of heating zone 2 through the horizontal ducts 48 and 49 (Figs. 2 and 4) discharging into the main 50 controlled by valve 51. Main 46 is provided with pressure gauge 52 by means of which the pressure obtaining at this point is indicated. Gases passing off through the main 46 are discharged into the quench tank 53. A liquid such as tar, may be supplied to the upper end of tank 53 through valved pipe 54. This liquid is restrained by transverse perforated plate 55 from which it is discharged downwardly in a large number of small streams. This liquid, together with any material condensed out of the gases entering through main 46, accumulates in base 56 of tank 53 up to the level indicated by line 57. Any excess over this may be continuously withdrawn through valved overflow pipe 58 passing through the cooler 59 in which it passes downwardly through pipes 60 carried in headers 61 and 62. A liquid may be passed into the space between headers 61 and 62 through pipe 63 passing off through pipe 64. From cooler 59, the liquid introduced through valved pipe 58 is diverted to storage through valved pipe 65. From tank 53, the gases supplied through main 46, less any constituents which may have been condensed in the tank 53, pass off through valved pipe 71 to pump 72 by which they are supplied to the mid-section of rectifying column 73. This column is spanned by a number of horizontal trays 74 equipped with bell caps and overflow pipes, not shown, for the purpose of dispersing any ascending vapor into the layer of liquid carried by each such tray. It is also equipped with a reboiler coil 75 in the base 76 and with a valved overflow pipe 77 by which liquid accumulating in the base over that necessary to maintain the level indicated by line 78, may be withdrawn.

From the upper end 81 of the rectifying column 73 gases are conducted away through pipe 82 communicating with condenser 83. In condenser 83, the gases move downwardly through tubes 84 carried in headers 85 and 86. Provision is made for cooling the gases in their passage through tubes 84 by the introduction of a coolant, such as water, through valved pipe 87 to the space between headers 85 and 86, passing off through valved pipe 88.

Condensate together with uncondensed gas passing off from condenser 83 moves downwardly through pipe 89 into the receiving tank 90. Any excess of condensate over that necessary to maintain the liquid level indicated by line 91 is continuously withdrawn through pipe 92. A part of this is recycled through valved pipe 93 by means of pump 94 discharging through pipe 95 into the upper end 81 of column 73, to serve as reflux in column 73. The balance is continuously withdrawn to storage through valved pipe 96. Bottoms accumulating in the lower end 76 of rectifying column 73 may be continuously withdrawn to storage through valved pipe 77. Uncon-

densed gas is withdrawn from tank 90 through valved pipe 97. Provision is made for the ascertainment of pressures obtaining in the heating zone by means of a number of pressure gauges, such as 101-106, spaced vertically along, and communicating with, the interior of heating zone 2.

Provision is also made for the ascertainment of temperatures obtaining in the heating zone by means of a number of temperature responsive devices such as shielded thermocouples 107-112 spaced vertically along transverse wall 35.

In the operation of the apparatus described, I first compound a suitable charge. One charge which I may use is compounded of the following materials: phosphate rock analyzing about 70% tricalcium phosphate or its equivalent in  $P_2O_5$  content, roughly two-thirds through 100 mesh and roughly 50% through 200 mesh; silica and coke breeze of roughly the same particle size as the phosphate rock; coal tar pitch M.P. 100° C. or higher, as determined by the cube in air method, coking value at least 40%.

These materials should be mixed in the following proportions:

|    | Parts               |
|----|---------------------|
| 25 | Phosphate rock..... |
|    | 360                 |
|    | Silica.....         |
|    | 120                 |
|    | Coke breeze.....    |
|    | 80                  |
|    | Coal tar pitch..... |
|    | 35                  |

30 The mix should be ball-milled for a period of hours to thoroughly incorporate the pitch with the remaining solid materials, following which it should be briquetted hot.

35 The charge which I prefer, however, is compounded of the same phosphate rock and silica together with bituminous coal which should run about 35% volatile as determined by conventional tests. These materials are mixed in the following proportions:

|    | Parts                |
|----|----------------------|
| 40 | Phosphate rock.....  |
|    | 360                  |
|    | Silica.....          |
|    | 120                  |
|    | Bituminous coal..... |
|    | 125                  |

45 The mix is ball-milled together for a period of at least 12 hours and until the coal has developed the property of flowing under relatively higher pressures. At this point the entire charge is briquetted under a pressure of about 15 tons per square inch. The briquettes so formed are strong and dense and may therefore be charged into the heating zone up to the level indicated by line 37, through the hoppers 33 and 35, by operation of bell valves 34 and 36. When this has been done, a carrier gas, such as carbon monoxide, is introduced through valved pipe 43 into base 41 of retort 1, at such a rate as to maintain positive pressure in the base, and the burners 8 and 21 are started in operation. During this stage valve 51 in main 50 is closed, and as soon as the temperature of pyrolysis is reached and thereafter the vapors produced are taken off through main 46 into quench tank 53, in which the heavier hydrocarbons are condensed by contact with incoming coal tar from 54, and the residual hydrocarbons, principally aromatics, are taken over into rectifying column 73. In column 73, by adjustment of the amount of reflux returned through line 95 and the amount of heat supplied through reboiler coil 75, these residual hydrocarbons are split into two cuts, i.e., heavier aromatics taken off from the base of the column through the valved pipe 77 and a lighter overhead consisting principally of benzol and toluol, which is taken off through valved pipe 82. Uncondensed gas is taken off through valved pipe 97.

70 Whenever a temperature of about 1000° C. is reached in the base 38 of the heating zone, the valve 51 in main 50 is partly opened and the phosphorous vapor, together with the carbon monoxide simultaneously produced by

reduction, are conducted away through main 50 to suitable condensers (not shown). At the same time, flow through main 46 is controlled by means of valve 71 and/or pump 72 at a rate which will carry the heavier products of pyrolysis overhead through main 46 and thereby prevent them from co-mingling with and contaminating the phosphorus simultaneously produced. One way of establishing this adjustment is to make provision for a continuous sampling of the phosphorus coming off through main 50 and to maintain such a flow through main 46, by means of pump 72, as is necessary to insure that this phosphorus will not show tar contamination.

Another way is to maintain such a rate of flow by means of the valve in pipe 71 and/or by means of pump 72 that the maximum pressure in that part of the heating zone above outlets 48 and 49 occurs at the 700-800° C. (preferably about 750° C.) temperature level. This will insure that products of pyrolysis generated above this level move upwardly, whereas those generated below this level move downwardly. Below this level, i.e., above this temperature, the products of pyrolysis are principally of lower molecular weight and in such limited amounts as not to seriously contaminate the phosphorus produced.

Whenever a temperature of 1260° C. is obtained in the base 38 of heating zone 2, the grate bars 39 are started in rotation for the continuous removal of exhausted charge. Simultaneously fresh charge is supplied intermittently by operation of bell valves 34 and 36 to maintain an upper level substantially at the line 37. In continuous operation the temperature at the level of outlets 48 and 49 should be held between about 950° C. and 1050° C. (preferably about 1000° C.) and the rate of rotation of the grate bars set to provide a residence time of at least 3 hours from the 1100° C. level down to the final level of about 1260° C. This will liberate about 95% of the phosphorus content of the ore. As heretofore explained, the rate of operation of the valve 71 and/or pump 72 is set to carry the heavier products of pyrolysis overhead through outlets 44 and 45.

In continuous operation the temperature adjacent the outlets 44 and 45 should be maintained between about 300-400° C., preferably about 350° C.

Of the products of pyrolysis passing off through main 46, as heretofore described, the tars are knocked down in quench tank 53 by contact with fresh tar introduced through valved pipe 54, and after passing through cooler 59 are carried off to storage through valved pipe 65. The remaining hydrocarbons passing off through valved pipe 71 and pump 72 into rectifying column 73 are split roughly into two fractions, i.e., an overhead fraction consisting principally of benzol and toluol, the excess of which over that recycled as reflux through line 95 is carried off through valved pipe 96, and a bottoms of heavier aromatics carried off through valve pipe 77.

I claim:

1. The continuous process of winning phosphorus from oxygenated ores containing the same which comprises mixing such an ore in particulate form with a carbonizing agent which becomes only plastic and not freely fluid up to the temperature of pyrolysis, thereby forming a mixture, said mixture containing sufficient carbon-yielding substance to form a coke in which the carbon is in excess over that consumable in the reduction of the  $P_2O_5$  and other reducible oxides present, thereafter briquetting said mixture, maintaining a charge of such briquettes in a vertically oriented heating zone with provision for top feed and bottom discharge, heating said charge in the upper portion of said heating zone out of direct contact with combustion gases to a temperature between about 350-1000° C. for a period of time sufficient to substantially complete pyrolysis, thereafter further heating said charge in the lower portion of said heating zone to a temperature of between 950 and 1050° C. at which reduction proceeds with the formation of carbon monoxide and phosphorus in gas phase

75

and phosphorus in gas phase and until at least a major part of the phosphorus content of said ore has been liberated, adding fresh briquettes to said charge at the upper end thereof and removing residual carbon and residual ore particles from said heating zone at the lower end thereof, conducting away said carbon monoxide and phosphorus in gas phase from said charge at an intermediate point and separately conducting away the heavier products of pyrolysis from said charge at a higher point.

2. Process according to claim 1 in which said carbon monoxide and phosphorus in gas phase are taken off from said charge between about a temperature level of 950-1050° C.

3. Process according to claim 1 in which said carbon monoxide and phosphorus are taken off from said charge at a temperature level of about the 1000° C.

4. Process according to claim 1 in which said heavier products of pyrolysis are taken off from said charge at a temperature level of between about the 300-400° C.

5. Process according to claim 1 in which said products of pyrolysis are principally taken off from said charge at a temperature level of about the 350° C.

6. Process according to claim 1 in which said carbon monoxide and phosphorus in gas phase are taken off from said charge at a temperature level of between about 950-1050° C., and said heavier products of pyrolysis are taken off from said charge at a temperature level of about between 300-400° C.

7. The continuous process of winning phosphorus from oxygenated ores containing the same, which comprises mixing such an ore in particulate form with a carbonizing agent which becomes only plastic and not freely fluid up to the temperature of pyrolysis, thereby forming a mixture, said mixture containing sufficient carbon-yielding substance to form a coke in which the carbon is in excess over that consumable in the reduction of the  $P_2O_5$  and other reducible oxides present, thereafter briquetting said mixture, maintaining a charge of such briquettes in a vertically oriented heating zone with provision for top feed and bottom discharge, heating said charge in the upper portion of said heating zone out of direct contact with combustion gases, to a temperature between about 350-1000° C. for a period of time sufficient to substantially complete pyrolysis, thereafter further heating said charge in the lower portion of said heating zone to a temperature of between about 950 and 1050° C. at which reduction proceeds with the formation of carbon monoxide and phosphorus in gas phase

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040

5045

5050

5055

5060

5065

5070

5075

5080

5085

5090

5095

5100

5105

5110

5115

5120

5125

5130

5135

5140

5145

5150

5155

5160

5165

5170

5175

5180

5185

5190

5195

5200

5205

5210

5215

5220

5225

5230

5235

5240

5245

5250

5255

5260

5265

5270

5275

5280

5285

<p

ucts of pyrolysis are principally taken off from said charge at about the 350° C. temperature level.

12. Process according to claim 7 in which said carbon monoxide and phosphorus in gas phase are taken off from said charge between about the 950-1050° C. temperature levels and said heavier products of pyrolysis are taken off from said charge between the 300°-400° C. temperature levels.

References Cited in the file of this patent

UNITED STATES PATENTS

|           |              |       |               |
|-----------|--------------|-------|---------------|
| 2,029,309 | Curtis       | ----- | Feb. 4, 1936  |
| 2,168,312 | Baily        | ----- | Aug. 8, 1939  |
| 2,675,307 | Klugh et al. | ----- | Apr. 13, 1954 |

FOREIGN PATENTS

|         |        |       |               |
|---------|--------|-------|---------------|
| 683,645 | France | ----- | June 16, 1930 |
|---------|--------|-------|---------------|